

Nov. 15, 1927.

1,649,741

S. RUBEN

ELECTRIC CURRENT RECTIFIER

Filed Sept. 22, 1924

*Fig. 1.*



*Fig. 3.*



*Fig. 4.*



*Fig. 5.*



Inventor

Samuel Ruben,

By Stewart & McKey

his Attorney

Patented Nov. 15, 1927.

1,649,741

# UNITED STATES PATENT OFFICE.

SAMUEL RUBEN, OF NEW YORK, N. Y., ASSIGNOR, BY MESNE ASSIGNMENTS, TO  
RUBEN RECTIFIER CORPORATION OF DELAWARE.

## ELECTRIC-CURRENT RECTIFIER.

Application filed September 22, 1924. Serial No. 739,188.

This invention relates to electrocurrent rectifiers and more particularly to an electrochemical rectifier of the dry contact-surface type.

5 Rectifiers of the above type are characterized by the use of an electrode of electro-positive material such as aluminum connected in circuit with another electrode through an intermediate layer of a sulphur compound 10 and depend for their operation upon the presence of a current blocking or rectifying film of one of the electrodes. Such rectifiers heretofore available have been low in efficiency and limited in their use to small currents, becoming unstable after a short period 15 of use.

The invention has for its object generally the provision of a rectifier of the dry surface contact variety which is free from the limitations mentioned above and is capable of 20 use over relatively long periods of time and has a sustained current output.

Other objects of the invention will in part be obvious and will in part appear herein- 25 after.

The invention accordingly comprises the features of construction, combinations of elements, and arrangement of parts, which will be exemplified in the constructions herein- 30 after set forth and the scope of the application of which will be indicated in the claims.

For a fuller understanding of the nature and objects of the invention reference should be had to the following detailed description 35 taken in connection with the accompanying drawing, in which:—

Fig. 1 is an axial, cross-sectional view of the invention embodied in the form of a cartridge fuse;

40 Fig. 2 is a circuit diagram showing the use of two of the rectifiers with a transformer and filter circuit for utilizing both halves of the cycle;

Fig. 3 is a modified form for use with 45 large currents;

Fig. 4 is a cross-sectional view of a series type in the form of a cartridge fuse with several rectifier elements in series for relatively high voltages; and

50 Fig. 5 is a diagram illustrating the method of forming a coating on one of the electrodes.

Referring to the drawings and first to Fig. 55 1, an electrode 1 of an electro-positive material, preferably one of aluminum, having

a coating of sulphide indicated at 2, is placed in contact with a second or electro-negative element in the form of a plate or disk shown at 3, and composed of cupric sulphide (CuS) and having its opposite face placed in contact with another element 4, which is a good conductor of heat and electricity, for example, brass. These constitute essential elements of the invention and may be given any physical form affording arrangement of 60 the different contacting surfaces in the order shown. In the present form the elements 1, 3 and 4 are mounted within a cylindrical casing 5 of insulating material, for example bakelite, threaded at its ends to take the 70 threaded terminal plugs 6 of suitable conducting material such as brass or copper, which through the interposed spring washer 7 hold the elements in place and in contact under constant pressure, compensating for 75 expansion and contraction of the parts due for example, to temperature changes.

In accordance with the preferred form of the invention a specially prepared sulphide coating is used on the electro-positive or 80 aluminum electrode. In rectifiers of the present general type heretofore proposed, it was found that the variable contact resistance at the rectifying film is the fundamental factor which prevents efficient or 85 practical operation. This variation in resistance at the rectifying film is due to the reaction which here takes place, namely, dry contact electrolysis, in which a film is formed by the passage of an inverse current 90 through the contacting surfaces of aluminum and a sulphur bearing compound. The density of the film thus produced is limited for the reason that just as soon as a slight film is formed it serves to prevent the further 95 formation of film. Regardless of how high an inverse potential is used in forming the film, the initially formed film is accompanied by a resistance product which insulates and reduces the inverse film forming 100 current to such a low value that the film necessary to withstand continuous alternating current operation cannot thus be formed.

It has been found that a coating of aluminum sulphide having the desired density may be formed on the aluminum electrode before assembling the elements by chemical process, and that the assembled rectifier unit with a coating formed will coat to impart substantially unilaterally conductive or recti- 105 110

fying properties without the necessity of first passing an inverse current for any material forming period, its alternating current operation being substantially constant without 5 sparking between the sulphide and the aluminum. The word density is here used, not in its restricted sense as meaning mass or specific gravity but, in a broad sense to indicate density, thickness or durability as to operating strength or resistance to over-load 10 break-down.

A method of producing this dense and efficient resistance coating consists in subjecting the aluminum electrode to a bath of 15 alkaline sulphide, such as sodium sulphide heated to about 100° C., the aluminum electrode being made the anode in a current path through the sulphide solution to a suitable cathode electrode such as brass or nickle, 20 which current is supplied from a suitable source with variable potential. The potential is increased with increasing strength or density of the coating up to a voltage higher than that used in the application of the unit. 25 A difference of potential of 35 volts will produce a coating of desired density. When the potential to be applied to the units is of low value, the electrolytic method of formation need not be used, since by boiling 30 the aluminum electrodes in a concentrated solution of sodium sulphide, a coating of sufficient density is formed, or where only a slight coating is sufficient, heating is not required.

35 The arrangement of apparatus for carrying out the electrolytic process of forming the coating is indicated diagrammatically in Fig. 5 in which 8 indicates a vessel of suitable heat-resisting and transparent material such as thin tempered glass for example, glass sold under the trade-name of pyrex, which vessel contains a concentrated solution of sodium sulphide in which the aluminum element 9 to be coated and a 40 cathode element 10 of brass or copper are immersed. The aluminum electrode 9 is connected through the conductor 11, milliammeter 12 and conductor 13 to the positive terminal of a variable potential battery 14, 45 while the anode element 10 is connected through conductor 15 to the variable contactor 16 adapted to engage different taps on the minus side of the battery 14. The purpose of the transparent container 8 is 50 to enable the physical condition of the coating to be observed during the progress of the coating process, and the purpose of the milliammeter is to indicate the electrical characteristics of the film during the process, 55 the potential being applied until the meter indicates a negligible current flow.

60

65 By the process of coating just described a pure sulphide coating may not be produced; it possibly contains more or less aluminum hydroxide. This however is not detrimental

as it does not alter beyond operating limits the resistance value of the coating desired to be obtained.

By the present invention the electronegative electrode element is a good electrical 70 conductor containing a sulphur component which is readily given up to the electropositive electrode element, here provided, whereby the rectifying film, upon injury, is immediately and automatically repaired by 75 the reaction electro-chemically produced at the junction of the electrode elements.

The electronegative electrode element is the intermediate element in the operative combination here shown, and is a disc having 80 a composition adapted to yield sulphur in this manner. Cupric sulphide (CuS) is a suitable material for its composition. Its use in the electronegative electrode element is thus an important feature of 85 the present invention, since it was found that a highly efficient and stable rectifier for use under practical conditions requiring a wide margin of safety as to over-load, extended use, etc., which could not be produced 90 with ordinary cuprous sulphide (Cu<sub>2</sub>S) as the electronegative electrode element. On the other hand, cupric sulphide (CuS) especially that produced by the method to be hereinafter described, has been 95 found to have the necessary qualities to satisfy commercial requirements.

In order to produce electrode elements of cupric sulphide, which have the improved electrical characteristics above described, a 100 preferred method consists in heating the copper in the form of a metallic copper plate of a thickness, preferably, of about 5 millimeters, in sulphur vapors in a non-oxidizing atmosphere at a temperature above 150 105 degrees centigrade, preferably about 450 degrees centigrade. Under this treatment substantially the entire copper plate becomes converted into a cupric sulphide plate, taking the form of a hard, dark blue to blackish, 110 solid, metal-like material, having conducting and other electrical characteristics, for example, a sufficiently low resistance which make it much superior to cuprous sulphide, (hemisulphide) or ordinary cupric sulphide 115 otherwise produced. In the method above described the thickness of the initial copper plate and the temperature at which it is exposed to the sulphur vapor, are important elements of the process. A temperature 120 above the minimum specified is found to be necessary to insure the prevention of the formation of cuprous sulphide (Cu<sub>2</sub>S) and yield the necessary solid cupric sulphide (CuS).

125 Using a pair of rectifiers constructed as described in the combination and arrangement of circuits and ancillary apparatus indicated diagrammatically in Fig. 2, the constants were as follows:

Area of rectifying film, 4 square square centimeters.

Output voltage of filter circuit, 6 volts.

Transformer ratio, step down, 10 to one.

5 Direct current resistance, in inverse connection, 1,000 ohms.

Direct current resistance, in conductive connection, .5 ohms.

Referring to the circuit connections of

10 Fig. 2 in detail, 20 is a step down transformer having its primary winding 21 connected with a commercial source of alternating current 22, in the present instance a 110-volt electric light and power circuit, and its

15 secondary winding 23, which is a split winding, connected through a filler circuit, consisting of the inductance 24 and condensers 25 and 25<sup>a</sup> with a pair of rectifiers 26 and 27. The terminals of the condensers 25 and 25<sup>a</sup>

20 are connected to the direct current output terminals 28 and 29 which in operation are connected or bridged by the desired direct current consumption device not shown. It will be seen that with the rectifying devices

25 26 and 27 connected to rectify in the direction indicated by the adjacent arrows, both sides of the cycle of the alternating currents induced in the winding 23 are rectified into unidirectional pulsating current which is

30 smoothed out into a substantially uniform direct current by the action of the inductance 24 and condenser 25.

In Fig. 3 is shown a form of the invention designed for commercial use where 35 large current capacity is required. This consists essentially of the same elements as that of Fig. 1, but with greater contact or operating area and with means for facilitating the radiation of heat. More especially

40 it comprises a central electrode 34 of copper, having both extended surfaces in contact with plates 33 of cupric sulphide (CuS) which in turn have their outer or remote faces in contact with a pair of aluminum

45 electrodes 31, the whole being clamped together by clamping bolts 36 and maintained under constant pressure by spring washers 37. The inner or contacting surfaces of the aluminum electrodes 31 are provided with a

50 coating of aluminum sulphide 32, while the outer faces are provided with flanges 38 to facilitate the radiation of heat. Where the central electrode 34 passes out beyond the lower clamping bolt 36 it is perforated with

55 an opening arranged to permit the bolt to pass therethrough without touching. A binding post 39 is mounted on the central electrode for making circuit connections therewith, while connection may be made 60 with aluminum electrodes through the lower bolt 36.

The arrangement of Fig. 4 is the same as that of Fig. 1 in all respects except that the group of elements 1, 3 and 4 is repeated a

65 number of times and the cylindrical casing

5 made sufficiently long to accommodate the increased number of groups. This arrangement is intended for use in relatively high potential circuits such as the standard 110-volt circuit without the use of a step down 70 transformer, the number of complete groups of elements varying according to the voltage.

In all the various forms of the invention it is important to have the contacting surfaces of the elements, especially the coated 75 surface of the aluminum and the adjacent or complementary surface of the cupric sulphide, ground to a uniform and polished surface.

While there is here shown and described 80 certain specific embodiments of the invention, it is to be understood that the invention is not limited to such specific embodiments but contemplates all such variants and modifications as fairly fall within the scope of 85 the appended claims. For example, the device may take any physical form, especially as to the arrangement of its terminals, enabling it to be readily substituted for other forms of current rectifiers, such as a two-electrode rectifier tube or a mercury-vapor tube, without disarrangement of the controlling circuits and ancillary apparatus, such as transformers, filter circuits and the like.

Having described my invention, what I 95 claim as new and desire to secure by Letters Patent is:—

1. An electric cell of the dry surface contact variety adapted for the rectification of alternating currents and the like, comprising 100 electropositive and electronegative electrode elements relatively widely divergent in the electrochemical series and disposed to maintain a continuously formed current blocking film therebetween; said electronegative electrode element comprising cupric sulphide.

2. An electric cell of the dry surface contact variety adapted for the rectification of alternating currents and the like, comprising 110 electropositive and electronegative electrode elements relatively widely divergent in the electrochemical series and disposed to maintain a continuously formed current blocking film therebetween; said electropositive electrode element comprising a body of aluminum, and said electronegative electrode element a body of cupic sulphide.

3. An electric cell of the dry surface contact variety adapted for the rectification of alternating currents and the like, comprising 120 electropositive and electronegative electrode elements relatively widely divergent in the electrochemical series and disposed to maintain a continuously formed current blocking film therebetween; said electropositive electrode element comprising a body of sulphide coated metallic aluminum, and said electronegative electrode element a body of cupric sulphide.

4. An electric cell of the dry surface con-

- 1 tact variety adapted for the rectification of alternating currents and the like, comprising electropositive and electronegative electrode elements relatively widely divergent in the 5 electrochemical series and disposed to maintain a continuously formed current blocking film therebetween; said electropositive electrode element comprising a body of metallic aluminum having a preformed resistance 10 coating, and said electronegative electrode element being a metallic compound having a surface adapted to react with said coating for current rectification and containing cupric sulphide.
- 15 5. An electric cell of the dry surface contact variety adapted for the rectification of alternating currents and the like, comprising electropositive and electronegative electrode elements relatively widely divergent in the 20 electrochemical series and disposed to maintain a continuously formed current blocking film therebetween; said electropositive electrode element comprising a body of metallic aluminum having a preformed coating of 25 aluminum sulphide, and said electronegative electrode element having a surface containing cupric sulphide adapted to react with the coating on said electropositive electrode element.
- 30 6. An electric current rectifying cell of the dry surface contact variety comprising an electropositive electrode element having a contacting surface of aluminum sulphide, and an electronegative electrode element of 35 cupric sulphide; said electrode elements being disposed for the continuous maintenance of an interposed asymmetric current blocking film.
- 40 7. An electric cell of the dry surface contact variety adapted for the rectification of alternating currents and the like, comprising electropositive and electronegative electrode elements relatively widely divergent in the electrochemical series and disposed to 45 maintain a continuously formed current-blocking film therebetween; said electropositive electrode element comprising a body of an electropositive metal having a preformed coating on one surface of a compound thereof, and said electronegative electrode element having a coating surface comprising
- cupric sulphide adapted to react with the coating on said electropositive electrode element.
8. An electric cell of the dry surface contact variety, adapted for the rectification of alternating currents and the like, comprising electropositive and electronegative electrode elements which are relatively electropositive and electronegative with respect to each other, and disposed to maintain an inverse current-blocking film at their contacting surfaces; the electropositive electrode element being a metal having a preformed coating containing a sulphide, the electronegative 65 electrode element comprising cupric sulphide.
9. An electric cell of the dry surface contact variety, adapted for the rectification of alternating currents and the like, comprising 70 electropositive and electronegative electrode elements which are relatively electropositive and electronegative with respect to each other, and disposed to maintain an inverse current-blocking film at their contact- 75 ing surfaces; the electropositive electrode element being a metal having a preformed coating containing a compound thereof, the electronegative electrode element comprising a maximum valent compound of copper 80 with sulphur whereby it is adapted to yield sulphur electrochemically to said film upon the passage of inverse current.
10. An electric cell of the dry surface contact variety, adapted for the rectification of 85 alternating currents and the like, comprising electropositive and electronegative electrode elements which are relatively electropositive and electronegative with respect to each other, and disposed to maintain an in- 90 verse current-blocking film at their contacting surfaces; the electropositive electrode element being aluminum having a preformed coating containing a compound thereof, the electronegative electrode element comprising 95 at maximum valent compound of copper with sulphur whereby it is adapted to yield sulphur electrochemically to said film upon the passage of inverse current.
- In testimony whereof I hereunto affix my 100 signature.
- SAMUEL RUBEN.